

Oct. 18, 1960

V. PULSIFER

2,956,320

CASTING OF METAL

Filed Dec. 28, 1955

2 Sheets-Sheet 1

FIG.1.



FIG.2.



INVENTOR:  
VERNE PULSIFER

By

John D. Willbina  
ATTORNEY.

Oct. 18, 1960

V. PULSIFER

2,956,320

CASTING OF METAL

Filed Dec. 28, 1955

2 Sheets-Sheet 2

FIG. 3.



INVENTOR:  
VERNE PULSIFER  
BY

*John T. Wilkins*  
ATTORNEY,

1

2,956,320

## CASTING OF METAL

Verne Pulsifer, La Grange, Ill., assignor to Olin Mathie-  
son Chemical Corporation, East Alton, Ill., a corpora-  
tion of Virginia

Filed Dec. 28, 1955, Ser. No. 555,923

10 Claims. (Cl. 22—57.4)

This invention relates to the art of casting of metals and more particularly to an improved apparatus and method for continuously casting a slab of metal in the cross sectional shape approaching that of strip or sheet metal. A typical slab may have cross sectional dimensions in the neighborhood from around 4" x 1/2" up to around 30" x 1/2" for example.

Heretofore, the method of continuously casting metals has met with a substantial degree of success only in casting of ingots of relatively great thickness. For this reason continuously cast circular ingots and rods or nearly square billets of relatively heavy sections are more common than rectangular sections having a width far in excess of the thickness. But it has long been recognized that it would be desirable to continuously cast a flat slab suitable for further processing to commercial sheet metal by just a few additional finish operations instead of the rather extensive rolling reductions, both hot and cold, and annealing steps required to bring a heavy slab or bloom down to the shape and gauge of the wrought strip or sheet metal product desired.

Attempts have been made to directly cast thin slabs of metal by continuously pouring molten metal between a pair of cooled rolls, e.g. U.S. 49,053, issued to Bessemer, and U.S. 382,321, issued to Norton et al., or upon the surface of a casting drum, e.g. U.S. 1,531,747, and U.S. 1,611,911, issued to Hazelett, or between co-operating drum and belt, e.g. U.S. 359,348, issued to Daniels, and even between traveling belts, e.g. U.S. 594,583 issued to Wood. But metal produced with the methods and devices of the type represented by this and other prior art and known improvements thereon has been inferior and commercially unacceptable except for a few low melting metals, notably lead and zinc. A metal such as cartridge brass or aluminum, for example, produced on apparatus of this type is found to be entirely too porous in internal structure and is characterized by a very poor surface having many cold shuts. These surface irregularities may be attributed largely to irregularities and disturbances in movement of the molten metal as it approaches the mold wall.

Therefore, one object of this invention is to provide a continuous casting apparatus and process free from the difficulties and disadvantages encountered with prior devices and novel methods of producing a comparatively thin continuous casting of metal slab.

Another object is the obtainment in continuous casting of substantial constancy of thermal conditions during the whole of the operation and of regularity of the progress of solidification by having as great and constant as possible a portion of the final cooling affected through the cross section of the ingot itself, with a thermal-gradient approaching the horizontal, rather than through the lateral surface of the ingot. Thus internal shrinkage and radial cracking are avoided to a considerable degree.

Another object is to provide a new and improved apparatus for economically and efficiently casting continu-

2

ous lengths of relatively thin metal metal strip of satisfactory soundness, surface quality and gauge.

Another object is the provision of new and superior means for the substantial elimination of mechanical forces and influences which disturb and impair the proper solidification of the molten metal in continuous casting apparatus of the type described.

A still further object is to provide a new and improved control of the molten metal solidification in continuous casting apparatus of the type described.

Other objects and advantages of the invention will be apparent from the following description and the accompanying drawing in which:

Fig. 1 is an elevational view in cross section of a preferred embodiment of this invention;

Fig. 2 is a view taken on II—II of Figure 1; and

Fig. 3 is a cross sectional plan view taken on line III—III of Figure 1.

In accordance with this invention the foregoing objects are accomplished by the provision of novel apparatus having a combination of coating features together adapted for improved continuous casting of a length of metal slab of a width far in excess of its thickness as will hereinafter more fully appear. The casting apparatus and process of this invention is characterized by an improved introduction of the metal and by an improved control of the solidification process.

One feature of the invention provides a metal shaping member in which substantially no relative motion occurs between the solidifying metal and the mold or die side walls defining the metal congealation regions of the apparatus. This is accomplished by forming the side walls of unidirectionally traveling surfaces of continuous, spaced apart metal belts or the like which support the molten metal during solidification and also by a particular structural arrangement of molten metal feed which prevents premature contact between the metal and the belts. This eliminates forces that might otherwise occur between the solidifying metal and the walls of the mold. By continuing the occurrence of metal solidification in the casting apparatus of this invention between traveling surfaces of adequate length there is avoided change of metal shape during solidification other than the normal contraction which always follows cooling of the metal. Cracks perpendicular to the longitudinal axis of the ingot are virtually avoided by substantially complete elimination of the restraint imposed by the mold.

Another feature relates to the capacity of the aforementioned particular structural arrangement of means for charging molten metal to the region of solidification not only without premature contact but also in a quiescent state and without exposure to other than a protective atmosphere. By this means there is avoided undesired heat loss prior to the point of solidification. To accomplish this the molten metal is introduced at the proper temperature from a relatively shallow pool under sufficient hydrostatic pressure into a region of confinement having a configuration substantially identical with and in collimation with the cross-section defined by the traveling side walls. This region is positioned to affect the metal immediately prior to entry of the molten metal into the metal shaping portion of the apparatus between the traveling side walls. Thus, rearrangement of the metal volume and the resulting disturbing flow of metal is substantially eliminated at the point of solidification. All disturbance of the metal both immediately prior to as well as during solidification is avoided in the casting apparatus herein described.

Another feature of this invention relates to interposition of a continuous coating or layer of mold dressing medi-

um of a desired and adjustable thickness and/or composition between the moving metal and the mold surfaces traveling in unison with the metal. The introduction of this medium has a number of functions, but the chief function is the control of the degree of heat transmission through the metal belts forming the mold side walls and regulation of the cooling rate for the casting process. Another is the provision of a reducing material in the mold about the metal as protection against oxidation. The dressing medium also functions as a seal between stationary and moving parts of the apparatus but not as a lubricant for the cast metal. No lubrication is required between the metal being cast and any part of the apparatus. A high degree of control of the casting process is obtained by the regulation of the thickness of this mold coating material functioning chiefly as an agency for controlling the heat transmission to the sidewalls. Furthermore, by means of this feature of the invention it is possible to not only adjust the mode of metal crystallization and to influence the metal structure forming between the flat faces of the slab but also to adjust the gauge of the slab within certain limits and from edge to edge. The latter prevents wedge shaped castings which are not desired in the rolling mill.

Cooling of the metal to solidification occurs chiefly through transmission of the heat by way of the solidified section of the casting which is subject to direct fluid cooling. Abstraction of heat longitudinally with respect to the molten metal at the point of solidification through the previously solidified cast metal is the essential means of cooling as compared to the heat lost laterally by way of the dressing media surrounding the metal and the metal belts forming the side walls of the die section of the apparatus. Ordinarily no other attempt is made to cool the rolls, belts or other parts of the apparatus at points at which molten metal is to be found in contact with the casting apparatus, except such cooling of the belts as is inherent to the device shown and described. However, the plastic dressing tends at first to have a relatively brief lateral cooling effect on the metal after which it acts as an insulator. This initial effect may be varied by heating or refrigerating the incoming dressing as desired for certain metals.

In the preferred embodiment described herein and illustrated in the accompanying drawing, the improved strip casting apparatus of this invention comprises a rigid supporting frame 1, carrying a main or discharge mold section 200 for imparting the desired cross sectional shape of the casting and an entry or upper mold section 100 for giving the molten metal a desired preliminary spatial arrangement and for feeding the molten metal to the other section under certain desired conditions. Supported on and journaled in the frame 1 are a first pair of face pinch rolls 2 and 3 and a first pair of side pinch rolls 4 and 5, which together with the face rolls 2 and 3 are the entry rolls. Also rotatably supported on the frame are a second pair of face rolls 7 and 8 and a second pair of side rolls the latter of which are not shown in the drawing but which are related to side rolls 4 and 5 as rolls 7 and 8 are to rolls 2 and 3. Movable supported on these rolls are two mold face belts 13 and 14 and two mold side belts 15 and 16. Disposed in the entry side of the bite of the first pairs of rolls but spaced by a predetermined distance, found suitable in practice, from the surfaces of the belts passing over these rolls is a hollow pouring block or tundish 17 adjustably supported on the frame saddle 18 mounted on frame 1. Housed in the saddle 18, in close association with the pouring block 17 and each of the first pairs of orifice defining rolls, are supply chambers 19, 20, 21 and 22 for feeding a plastic mold dressing material 23 between each of the belts and the pouring block. Also mounted on the frame saddle 18 is any suitable adjustable means for varying at will the opening between surfaces of the belts 13, 14, 15 and 16 and the block 17

and thereby controlling the thickness of dressing material fed therefrom in interposed relationship between each of the traveling mold belts and the metal of the casting.

5 The sizing pass 26 of mold section 200 is generally defined by the complementary mold face belts 13 and 14 and the complementary mold side belts 15 and 16. These at pass 26 support the molten metal in its transition to the solid state without relative motion between the solidifying metal and the surrounding belts and also aid in influencing the heat abstraction desirably. A pass length at least adequate to accomplish the foregoing is selected.

10 The belts 13, 14, 15 and 16 are carried about the pair of rolls 2 and 7, pair 3 and 8, pair 4 and 9 and pair 5 and 10 respectively. The rolls are driven in unison in any suitable manner. To assure that all belts move at the same speed together, each group of rolls is interconnected as by bevel gears 6.

15 Each belt is preferably a thin continuous band of metal such as stainless steel. The bridging parts of the belts coming from each one of the confronting faces of the first pairs of rolls, and taken up on a corresponding one of the confronting faces of the second pairs of rolls are maintained by any suitable means at sufficient tension to cause these parts of the belts to travel in straight lines between each of the two respective rolls on which each belt is supported and operated. These straight line portions of the belts adjacent the lateral edges thereof are disposed in a contiguous relationship with respect to each other such that together the belts form the four traveling side walls of a generally rectangular passageway or cavity into which the molten metal is teemed directly from the pouring block 17 and it is in this substantially rectangular cavity that the shaping or molding of the casting occurs.

20 The mold face belts 13 and 14 which correspond to and confine the wide flat faces of the strip to be cast, are broad and flat as compared to the relatively narrow mold side belts 15 and 16.

25 In order that the side belts may better fit in sealing relationship against the spaced parallel mold face belts 13 and 14, each of the side belts preferably is provided with a concavity by running the relatively narrow side belts around pairs of concave faced side rolls including rolls 4 and 5 each of which has a face width somewhat less than the width of the flexed mold side belts in order that the edges of the side belts may extend somewhat beyond the side pinch rolls whereby the side belt edges are adapted to be forced into spring pressure contact with the mold face belts. This concave shape of mold side walls gives a desirable convex or rounded edge contour to the casting and tends to reduce severe corner cooling which introduces unequal contraction and may result in splitting of the casting.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 977

the block 17 and the orifice defining rolls. This spout 32 encloses a mold entry passageway 33 having surfaces defined by the parallel straight lines tangent to the aforementioned rectangular mold sizing pass 26 defined by the belts as they pass over the first set of rolls. This rectangular passageway serves to lead the molten metal under desired confinement within the block from the reservoir 31 to the zone of congelation between the belts 13, 14, 15 and 16 not only without exposure to the atmosphere but also without premature lateral cooling and freezing with the concomitant undesirable formation of a curvilinear metal "skin" that would ordinarily be formed in the absence of mold section 100 and immediately thereafter undergo disruption beyond the roll pass or bite to make a strip having as a consequence an inferior quality. Further the passageway 33 serves to give the molten metal a preliminary "shape" like that of the final casting so that subsidence of metal cross flow, counterflow and turbulence may occur in the passageway 33. The spout portion 32 of the block 17 extends as close as possible to the sizing pass 26 defined by the closest approach of the surfaces of the four belts riding the entry rolls at the bite of these rolls. By means of this particular block structure there is prevented the inception of freezing or solidification of the molten metal on the converging faces of the mold face and side belts at the rolls before the metal has reached a point at the aforementioned "orifice." The prevention of freezing on the interior walls of an open ended traveling belt type of continuous casting mold prior to movement of the metal to a place in the mold having the desired constancy of shape is an important factor together with the other features of the invention in securing a high quality continuously cast slab of metal.

While the block 17, forced by any suitable means to ride in juxtaposed relationship adjacent the dressing medium on the moving belts, has been described as feeding metal vertically downward, it is evident that the apparatus may be modified to operate horizontally or even to feed the metal upwardly. The depth of the reservoir 31 is not limited to the radius of the rolls and is made adequate to exert enough pressure to resist gas release and the resultant porosity in the metal.

At the point of transfer of the quiescent molten metal from the passageway 33 in the block 17 to the main mold section 200 between the traveling mold belts, there is fed by extrusion a thin peripheral layer of semi-solid mold dressing medium 23 of controlled anti-oxidant and preferably thermally insulating composition, of suitable plasticity and of controlled thickness between the molten metal and the belts. A suitable medium may consist of one or more of carbon black, graphite, bone ash, magnesium oxide, asbestos, vermiculite, kieselguhr, or diatomaceous silica or porous silica gel sold under the trademark Sil-O-Cel in any suitable vehicle such as kerosene, lard oil, or a silicone. The medium is compounded to give suitable properties and a small but desired amount of inert or at least reducing atmosphere under the various conditions encountered in the casting operation. The dressing applied to the mold face belt 13 may be identical with the dressing applied to the opposing mold face belt 14 but also may be of different composition in some cases to facilitate crystallization control in the casting. The dressing applied to the mold side belts 15 and 16 as a rule should be of a more heat insulating nature than the dressing applied to the face belts which may be accomplished in the former by a high content of kieselguhr, bentonite or the like. With appropriate subdivision of each chamber, different dressing may be applied to the same belt. The dressing layers from all supply chambers together form a thin sheath 41 surrounding the periphery of the metal and serves as a conductor of heat of controlled resistivity to the lateral flow of heat from the metal being cast to the bands of metal between which solidification takes place.

The element of control is effectuated chiefly by varia-

tion in the thickness of the thin extruded layer 41 of dressing compound carried by the belts. While it is preferred that the thickness of the dressing layer 41 be less than or at most not greatly in excess of about 0.005 of an inch, the thickness is to be varied by the mold operator until there is achieved the desired casting quality and thickness as hereinbefore explained. The thickness of dressing will, of course, vary with the composition of the metal cast, with the composition of the dressing, with the temperatures of the charging metal and coolant employed and also with other factors such as variations in the thickness, cross sectional area and speed of the strip of metal being cast.

As a further means of controllably varying the heat transmission via the belts and to improve the dressing carrying capacity thereof the belt surface facing the casting cavity may be provided with an adherent film of oxide or phosphate or the like. The same surfaces of the belts may also be initially scratch brushed to an extent insufficient to increase the heat transmission capacity thereof seriously but sufficient to aid initial adherence of the dressing medium to the belts. With a suitable dressing a network of scratches in the belt surfaces may provide a replica surface on the casting responsible for more rapid removal of heat by way of the emerging casting.

For varying and holding the spacing of the pouring block 17 from the surfaces of the mold face and side belts and thus for varying the dressing charging opening or gate circumscribing the casting metal at the points where passageway 33 in mold section 100 terminates and main mold section 200 begins, there is provided on each side any suitable means such as screw-down rods 35, the internally threaded helical gear 36, the equalizer rod 37 with screws 38, the internally threaded helical gear 39 with hand wheel 34, and compression springs 40.

Alternately, there may be provided a number of wedge cams carried by the frame 18 for adjustably supporting the block 17, it being yieldably urged toward the bite of the first pairs of pinch rolls by suitable means such as springs. Such wedge cams would be adapted to coact with corresponding cam following surfaces formed in block 17 as the cams are operated by suitable manually controlled means such as lead screws. However, it is to be understood that other means equivalent to the screw-down means shown or the cam means referred to may be substituted therefor. In any event such means for one side may be operated either at substantially equal or different rates with respect to the means for the other side.

Dressing material 23 is carried in arcuately shaped supply chambers having walls extending from the saddle 18. Each chamber has opposing lateral walls contiguous with one of the belts and is open on an arcuate side at the belt with which it is associated. Although one chamber is shown for each belt, it will be appreciated that there may be a plurality. As a means for urging the plastic dressing medium from the supply chambers 19, 20, 21, and 22 into the space between the convex surfaces of the mold belts and the complementary concave surface of the block 17 and for injecting the dressing as a thin sheath on the belts about the molten metal from the circumscribing orifice at the point where the molten metal leaves passageway 33 in the block 17 and enters the sizing pass 26 and straight walled portion of the traveling belt mold section 200, there is provided in association with each dressing supply chamber a fluid pressure operated ram 50 pivotally supported at one end on the frame 1 and connected at the other end to pistons 51 having suitable arcuate sides to ride the belt and fit the roll surface embracing chambers. This construction is especially advantageous for the belt-over-rolls type of casting machine of this invention.

Congelation of the metal occurs in the moving sheath of dressing material borne by the belts traveling in unison with each other and the metal being cast.

Cooling of the metal to solidification in the final stage of latent heat abstraction is accomplished primarily by drastic longitudinal heat transmission through the solidified ingot 42. This is preferably done by means of jets of cooling water issuing from a plurality of nozzles 45 positioned adjacent the delivery end of mold section 200 immediately opposite the belts passing over the second or discharge sets of rolls 7, 8, 9 and 10. High pressure cooling water directed between the emerging casting 42 and the coated belts results in a profuse and turbulent flow of the coolant over the casting surface which is large for a rectangular slab shape case as compared to the volume of the casting, thus effecting a comparatively rapid abstraction of heat therefrom. Furthermore, impingement of the high pressure jets of water serves to cleanse both the belts and the ingot of adhering spent dressing material, and to replenish the immersion bath 46 with a stream of cooler liquid replacing the warmed liquid discharged. The resulting longitudinal abstraction of heat is proportioned as needed in the early stages of metal cooling with a variable portion of lateral heat abstraction which rapidly becomes minor as the metal progresses through section 200.

In the device of this invention, collimation of all parts of the molten and solidified metal undergoing casting is achieved as is the avoidance of any disruption of the crystallization process from disturbances caused by bending or vibratory forces, which would be set up by lateral misalignment. This is done by supporting both the entry and the discharge rolls of mold section 200 in the rigid frame 1 and by nesting the pouring block 17, of the particular structure shown and described, in form fitting relationship just ahead of the bite of the entry rolls. By the supporting system here disclosed alignment between sections 100 and 200 of the casting apparatus is maintained and undesired movement and bending between the solid casting 41 and the molten metal at the zone of congelation in sizing pass 26 is prevented.

The general operation of the casting apparatus and method of this invention should be readily understood in view of the foregoing description, but may be described together briefly as follows: In operation, first of all, molten metal is teemed into block 17 of mold section 100 to maintain the desired level of the reservoir 31 from which liquid metal at a desired temperature is fed to passageway 33 of down spout 32. Here, the molten metal under hydrostatic pressure arranges itself to the desired spatial shape, and turbulence in the flowing stream has an opportunity to subside. From passage 33 the metal enters the sizing pass 26 between the belts of mold section 200 where the metal encounters the refractory dressing material 23 being extruded in a layer 41 of desired thickness, composition and temperature for the metal being cast. In this traveling lateral sheath, the heat of the metal is abstracted at first laterally over a small portion of travel of metal, belts and the dressing layer. As the lateral cooling effect diminishes rapidly, the longitudinal cooling effect of cooling sprays 45 and coolant bath 46 becomes stronger. At this point in the process, dressing layer 41 operates as a heat insulating sheath. The resultant cooling in ingot 42 is manifested by gently curved isotherms approaching the horizontal instead of the deeply curved isotherms which are accompanied by an extremely high gradient especially at the lateral surfaces of many heretofore continuously cast ingots. Thus, while the metal is in sizing pass 26 of mold section 22, an excessively rapid succession of isotherms is avoided. In sizing pass 26 the metal is supported adequately in its transition to the solid state during which it is subjected to no change of shape as occurs on prior casting machine with rolls or drums. Furthermore, there is no relative motion between metal and the mold so that frictional restraint, cold shuts and cracking perpendicular to the ingot axis are avoided.

As the solid metal 42 with desirable external shape and internal structure emerges from pass 26 substantially

all of its surface is subjected to strong cooling by sprays 45 and quench bath 46. At this point the casting process has progressed sufficiently so that there is no danger of impairment of the metal by the quenching. At the same time the belts 13, 14, 15 and 16 of the apparatus are cleaned off in condition for another cycle through dressing supply chambers 19, 20, 21 and 22.

The apparatus and process are admirably adapted to automatic control. The speed of the casting, feed of the dressing medium, and both the temperature and impingement of quenching liquid at 45 and 46 may be interlockingly controlled by any suitable sensory control equipment which may be associated with the apparatus described.

From the foregoing description it is obvious that one advantage secured by means of the apparatus and process of the present invention is that the moving metal begins solidifying at points substantially all equally remote from the point at which the molten metal is charged to the mold and solidification proceeds directionally in a controlled manner toward the charging point with a minimum of hindrance by lateral solidification whereby shrinkage voids and serious bridging are virtually eliminated even in the case of alloys having a wide freezing range. Further, by means of the present invention, although an extremely shallow freezing crater is obtained, uncontrolled penetration by the incoming stream of molten metal from the charging point is prevented since the momentum and turbulence of the stream is eliminated and as a consequence the solidifying metal has a minimum of gas carried down into it and washing contact with liquid metal is prevented. Especially this invention is directed to producing ingots reasonably free from surface cracks, segregation, and internal disruptions all of which are known to occur when metal is chill-cast on and subjected to squeezing action between the converging surfaces encountered in prior casting devices of the roll type.

While the invention has been described without reference to any particular metal, any suitable metals such as copper, aluminum, magnesium and steel and their alloys may be continuously cast with advantage by means of the apparatus and process described herein. Although with some modification linked sections may be used in lieu of the belts, endless belts of either solid, stranded or woven construction are preferred because of the smooth surface obtainable on the ingot, the reduction possible in the bulk of the apparatus, as well as the unique suitability of belts to the entire design.

Since other embodiments may occur to those skilled in the art, it is to be understood that various modifications may be made in the invention described without departing from the spirit thereof and that the foregoing is intended to illustrate a preferred embodiment and not to limit the scope of the present invention except as set forth in the appended claims.

What is claimed is:

1. An apparatus for the continuous casting of metal in a rectangular cross sectional shape having a width far in excess of the thickness thereof comprising a rigid frame, at least a pair of associated entry rolls in spaced elongated parallel relationship, a corresponding second pair of discharge rolls in line with said entry rolls but longitudinally spaced therefrom, said rolls being rotatably mounted in fixed spaced relationship with respect to each other on said frame, a pair of short entry rolls together with a pair of short discharge rolls each pair of which is arranged in spaced parallel relationship with respect to each other and transverse to said arrangement of elongated entry rolls and discharge rolls respectively, endless belts each mounted to travel between one roll of said first pair and one roll of said second pair of rolls in spaced parallel relationship between the movable confronting portions of said entry and second pair of rolls, said rolls and belts defining a rectangular sizing pass adapted to travel with and shape the metal, means for feeding

molten metal to said sizing pass, said means extending into the space between said belts at the confronting portions of said entry rolls and having outer concave surfaces complementary to the contour of the converging part of said rolls and traveling belts and terminating in proximity to the point of minimum spacing between said entry rolls, means for mounting said metal feeding means in spaced relationship with respect to the portion of the belts traveling over the entry rolls, said extending portion of the feed means having a passage for feeding the molten metal in a cross sectional area and shape substantially identical with the cross sectional area and shape of said sizing pass, and means for continuously feeding a layer of dressing medium to said pass and between each of said belts and the metal issuing from said passage.

2. The apparatus of claim 1 having means for applying a high velocity stream of cooling fluid directly to substantially all of the surfaces of the solid metal shape immediately upon its emergence from the sizing pass adjacent the discharge rolls at an angle so as to direct said stream into impingement with the metal at the point of divergence of the belts from said discharge rolls so as to obtain maximum cooling of said casting and said belts.

3. The apparatus of claim 1 wherein the means for mounting the metal feeding means is adjustable so as to vary the thickness of the layer of dressing medium carried on the belts into the sizing pass.

4. The apparatus of claim 2 wherein the means for mounting the metal feeding means is adjustable and wherein the means for applying cooling fluid is also adjustable, whereby desirable proportioning of both lateral and longitudinal heat abstraction is obtained.

5. In apparatus for the continuous casting of metal, a pair of spaced rolls and belts converging over a portion of the surface of said rolls and passing through and beyond the bite of said rolls in spaced parallel relationship to define a sizing pass, means for distribution of molten metal to said sizing pass, said distribution means having outer concave surfaces complementary to the contour of the converging portion of the belts and an internal passage in collimation with said sizing pass and of cross section substantially identical with the cross section of the sizing press, and means for feeding a layer of dressing medium of desired thickness between said opposed surfaces of the belts and the metal being cast in the sizing chamber, said last means comprising an arcuately shaped dressing supply chamber mounted with an arcuate open side adjacent the surface of each of said belts at its roll, a positioner for spacing said concave surface from said portion of the belt on the roll whereby a dressing feed gate orifice is established between said supply chamber and sizing pass, and a piston for extruding dressing material from said supply chamber from said gate orifice into the sizing pass as layer on each of said traveling belts.

6. Apparatus for the continuous casting of metal in a rectangular shape having a width in excess of the thickness thereof comprising coacting sidewalls completely surrounding an open ended congealing cavity and moving in unison with said metal being cast, said side walls consisting of a pair of relatively broad face belts in relatively closely spaced substantially parallel, opposed relationship and a pair of relatively narrow side belts in relatively remotely spaced substantially parallel opposed relationship, said side belts being concavely shaped with respect to said cavity and having lateral edges maintained in contiguity with the opposed surfaces of said face belts inwardly from the lateral edges of the face belts.

7. The apparatus of claim 6 including means for applying a desired thickness of dressing medium to the interior surfaces of said belts. 70

8. The apparatus of claim 7 wherein the means for applying dressing medium consists of a dressing supply chamber having a gate adjacent each belt at the rolls and a piston for extruding the medium through said gate over the belt.

9. The method of continuous casting of metal comprising feeding molten metal into a first mold portion under low hydrostatic pressure of a shallow pool of the metal with a minimum of turbulence to form a confined stream having both a cross sectional and axial shape substantially identical with that of the solidifying metal, for a substantial distance in the axial casting direction whereby the stream is maintained substantially turbulence free, applying a plastic mold dressing medium to the wall of a second mold portion continuous to the first and moving axially to form a peripheral sheath laterally of the metal while adjusting the thickness of said sheath and simultaneously feeding said stream to initially cool and congeal it within said predetermined thickness of sheath traveling in unison with the metal being cast, and thereafter applying a cooling agent to the surface of the ingot substantially immediately upon its emergence from said second portion, thereby abstracting heat from the metal axially at all times during casting and laterally only by initial contact of the metal and sheath at a rate controlled by said dressing.

10. In apparatus for the casting of metal in a continuous length, open-ended metal shaping means having straight side walls traveling with the metal being cast, means separate from said shaping means for feeding the molten metal between straight walls directly to said metal shaping means substantially without turbulence and in the final cross sectional shape and with a straight axis identical with that of said metal shaping means for a substantial distance in the direction of casting, means for variably spacing said shaping means and feeding means, and means for interposing through said space a thickness of traveling dressing medium between the side wall of said shaping means and the metal so that said thickness is controlled in correspondence with said spacing, said side walls and dressing medium traveling in unison with the metal being cast.

#### References Cited in the file of this patent

| UNITED STATES PATENTS |                 |                                     |
|-----------------------|-----------------|-------------------------------------|
| 45                    | 379,096         | Brooke ----- Mar. 6, 1888           |
|                       | 441,643         | Close ----- Dec. 2, 1890            |
|                       | 594,583         | Wood ----- Nov. 30, 1897            |
| 50                    | 1,321,658       | Mellen ----- Nov. 11, 1919          |
|                       | 2,108,753       | Low ----- Feb. 15, 1938             |
|                       | 2,128,941       | Hudson ----- Sept. 6, 1938          |
|                       | 2,131,070       | Poland ----- Sept. 27, 1938         |
|                       | 2,169,893       | Crampton et al. ----- Aug. 15, 1939 |
| 55                    | 2,171,132       | Simons ----- Aug. 29, 1939          |
|                       | 2,183,010       | Coxe ----- Dec. 12, 1939            |
|                       | 2,225,373       | Goss ----- Dec. 17, 1940            |
|                       | 2,242,350       | Eldred ----- May 20, 1941           |
|                       | 2,348,178       | Merle ----- May 2, 1944             |
| 60                    | 2,527,545       | Goss ----- Oct. 31, 1950            |
|                       | 2,560,639       | Giesler et al. ----- July 17, 1951  |
|                       | 2,640,235       | Hazelett ----- June 2, 1953         |
|                       | 2,770,022       | Brennan ----- Nov. 13, 1956         |
|                       | 2,790,216       | Hunter ----- Apr. 30, 1957          |
| 65                    | FOREIGN PATENTS |                                     |
|                       | 703,269         | Great Britain ----- Feb. 3, 1954    |
|                       | 108,184         | Australia ----- Aug. 4, 1939        |
|                       | 813,755         | Germany ----- Sept. 17, 1951        |